

June 28, 1932.

H. L. PELZER

1,865,206

## ART OF CRACKING HYDROCARBONS

Filed Dec. 16, 1929



INVENTOR  
Harry L. Pelzer  
BY  
Pennie, Davis, Marvin & Edwards  
ATTORNEYS

## UNITED STATES PATENT OFFICE

HARRY L. PELZER, OF HIGHLAND, INDIANA, ASSIGNOR TO SINCLAIR REFINING COMPANY, OF NEW YORK, N. Y., A CORPORATION OF MAINE.

## ART OF CRACKING HYDROCARBONS

Application filed December 16, 1929. Serial No. 414,356.

This invention relates to the manufacture of motor fuel gasoline having a high critical compression.

The invention is of special value in conjunction with cracking operations in which high boiling hydrocarbon oil is heated to a high cracking temperature in the vapor phase for the production of gasoline, such for example as are described in my application filed June 13th, 1927, Serial Number 198,621, but the invention is also useful in conjunction with other types of cracking operations in which high boiling hydrocarbon oil is heated to a high cracking temperature, upwards of 950° F.

I have discovered that the products of the reaction between sulfuric acid and the unsaturated hydrocarbon constituents of the gas mixtures produced in such cracking operations include at least two types of constituents, the addition of which to gasoline fractions imparts to the resulting gasoline mixture a higher critical compression. One such type of these reaction products includes oxygenated compounds of alcohol, aldehyde or ketone character, and another such type of these reaction products includes compounds formed as a result of polymerization of these unsaturated hydrocarbon constituents.

According to this invention, a high boiling hydrocarbon oil, higher boiling than gasoline, is subjected to a cracking temperature upwards of 950° F. and a gas mixture including unsaturated hydrocarbon constituents is separated from the products of the cracking operation, a hydrocarbon composite including the unsaturated hydrocarbon constituents of this gas mixture is subjected to treatment with sulfuric acid, the reaction products of this treatment are separated into two parts, a composite acid mixture and a composite oil mixture remaining immiscible with the acid mixture, a polymerized gasoline fraction is distilled from the separated composite oil mixture, the separated composite acid mixture is subjected to hydrolysis to produce a second composite oil mixture and an oxidized gasoline fraction is distilled from this second composite oil mixture. Either or both of the composite polymerized gasoline

fraction and the composite oxidized gasoline fraction so produced may be combined with the gasoline condensate produced in the same cracking operation or with other gasoline fractions, or either or both of the composite polymerized gasoline fraction and the composite oxidized gasoline fraction may together with the gasoline condensate produced in the said cracking operation be combined with other gasoline fractions to produce a motor fuel gasoline having a high critical compression.

The invention will be further described in connection with the accompanying drawing, which illustrates, diagrammatically and conventionally, one form of apparatus adapted for carrying out one embodiment of the process of the invention.

The receiver 1 of the apparatus illustrated in the accompanying drawing is connected through connection 18 to the condenser of apparatus in which a high boiling hydrocarbon oil, such as gas oil or kerosene for example, is subjected to a cracking temperature upwards of 950° F. For example, the receiver 1 may correspond to the receiver "93" connected to the condenser "84" in the apparatus illustrated in my application filed June 13th, 1927, Serial Number 198,621.

The gasoline condensate and the associated gas mixture produced in the cracking operation are discharged into the receiver 1 through connection 8. An initial separation between the gasoline condensate and the gas mixture including uncondensed vapors is effected in this receiver. The gasoline condensate separated in the receiver 1 is pumped through connections 9 and 12 by means of pump 3 into the upper end of the scrubbing tower 4, and the gas mixture separated in the receiver 1 is forced through connections 13 and 14 by means of compressor 2 into the lower end of the scrubbing tower 4, a pressure being maintained in the scrubbing tower 4 materially higher than the pressure maintained in the receiver 1. The scrubbed gas mixture is discharged from the upper end of the scrubbing tower 4 through connection 15. The condensate mixture including unsaturated hydrocarbon constituents absorbed

from the gas mixture in the scrubbing tower 4 is discharged through connection 16 to the rectifying tower 5. This rectifying tower may be operated under a pressure intermediate that maintained in the receiver 1 and that maintained in the scrubbing tower 4, or under a pressure approximating that maintained in the scrubbing tower 4. A vapor mixture containing in high concentration 10 unsaturated hydrocarbon constituents absorbed from the gas mixture subjected to scrubbing treatment in the scrubbing tower 4 is discharged from the upper end of the rectifying tower 5 through connection 17 into the condenser 6. The condensate from this condenser is discharged into the receiver 7. Any gas remaining uncondensed is recycled through the scrubbing tower 4 by means of connection 18. The condensate collecting in the receiver 7 containing unsaturated hydrocarbon constituents, such as propylene, butylene, amylene and in some cases even ethylene, in high concentration, is supplied to the mixing pump 10 through connection 19. The rectifying tower 5 is shown as provided with a cooling coil 20 and a heating coil 21 for purposes of control. A part of the condensate collecting in the receiver 7 may also be reintroduced into the upper end of the rectifying tower 5 through connection 22 for purposes of control. A rectified gasoline condensate is discharged from the lower end of the rectifying tower 5 through connections 45 and 47 and cooler 46.

In the cracking operation, the high boiling hydrocarbon oil may be heated to a cracking temperature in the range 950-1200° F., for example, under a pressure in the range 0-500 pounds per square inch, for example. The receiver 1 may be operated under atmospheric pressure or under some higher pressure. The scrubbing tower 4 may be operated, for example, under a pressure upwards of 50 pounds per square inch higher than the pressure maintained in the receiver 1 and up to 500 pounds per square inch or more, for example. The rectifying tower 5 may be operated under a pressure approximating that maintained in the scrubbing tower 4 or under some lower pressure.

The condensate containing unsaturated hydrocarbon constituents in high concentration supplied to the mixing pump 10 through connection 19 is, in the mixing pump 10 and the conduit 23, subjected to treatment with strong sulfuric acid supplied through connection 24. The length of the conduit 23 may be adjusted to provide an appropriate period of contact between the reacting materials, and the reacting materials may be maintained under a pressure in the conduit 23 higher than that maintained in the separating tower 11 by means of valve 24. A part of the acid mixture collecting in the separating tower 11 may be recirculated by means of connection 25 through the mixing pump 10 and the conduit 23 together with fresh acid supplied through connection 24 and condensate supplied through connection 19. The separating tower 11 is shown as provided with a cooling coil 39 for purposes of control. The composite acid mixture and the composite oil mixture remaining immiscible with the acid mixture produced as a result of the reaction effected in the mixing pump 10 and the conduit 23 are separated in the separating tower 11, the composite acid mixture being discharged through connection 26 and the composite oil mixture through connection 27. Any gas mixture remaining is discharged through connection 28. The composite oil mixture discharged through connection 27 is supplied to the still 29, to which a neutralizing agent may also be supplied through connection 30, and a composite polymerized gasoline fraction is distilled from this oil mixture therein, this composite polymerized gasoline fraction being condensed in the condenser 31 and discharged through connection 32. The composite acid mixture discharged through connection 26 is subjected to hydrolysis, in the mixing pump 33 and the conduit 34, with water supplied through connection 35. The products of this hydrolysis are discharged into the fractionating tower 36, in which the lower boiling components of these products are distilled from the diluted acid mixture to form a second composite oil mixture condensed in the condenser 37. The fractionating tower 36 is provided with a heating coil 38 for effecting this distillation. The diluted acid mixture is discharged through connection 39, for example, to concentration apparatus from which strong acid may be returned to the mixing pump 10 through connection 24. The second composite oil mixture, condensed in the condenser 37, is supplied through connection 40 to the still 41, to which a drying agent may also be supplied through connection 42, and a composite oxidized gasoline fraction is distilled from this second oil mixture therein, this composite oxidized gasoline fraction being condensed in the condenser 43 and discharged through connection 44.

The reaction between the sulfuric acid and the condensate containing unsaturated hydrocarbon constituents in high concentration, effected in the mixing pump 10 and the conduit 23, is advantageously carried out under a pressure high enough and at a temperature low enough to maintain the hydrocarbons present substantially in liquid phase. Sulfuric acid of strength corresponding to 50-100 per cent.  $H_2SO_4$ , for example, may be used; however, stronger acid promotes polymerization and it is in general more advantageous to use sulfuric acid of a strength corresponding to upwards

of 80 per cent.  $H_2SO_4$ . Higher temperatures also promote polymerization, but at higher temperatures the pressures become excessive; the reaction may be effected satisfactorily at temperatures in the neighborhood of 60-90° F. The proportion of sulfuric acid used may vary widely depending upon the concentration of unsaturated hydrocarbon constituents in the treated condensate, but in general a volume of sulfuric acid corresponding approximately to that required theoretically to form sulphates of the unsaturated hydrocarbon constituents present is an appropriate proportion. The proportion of water used in the hydrolysis may vary, for example, from 25 per cent. to 500 per cent. of the sulfuric acid used.

Solutions or suspensions of caustic soda or hydrated lime in oil or oil-water mixtures may be supplied to the still 29 through connection 30 as neutralizing agents. Caustic soda, hydrated lime, and calcium carbide, are useful as a drying agent in the still 41 and may be supplied thereto through connection 42 in suspension in oil. A gasoline fraction may also be supplied to the still 41 through connection 42 as a drying agent for drying the distillate discharged through connection 44. The stills 29 and 41, for example, may be arranged and operated generally as described in Letters Patent Number 1,639,531, issued to Sinclair Refining Company, August 16th, 1927, on an application of Ernest B. Phillips and James G. Stafford.

The rectified gasoline condensate, the composite polymerized gasoline fraction and the composite oxidized gasoline fraction are discharged, in the apparatus illustrated, through connections 37, 42 and 44, respectively, and the manifolded connections 48, 49 and 50, for combination with each other or with other gasoline fractions, for the production of motor fuel gasolines having a high critical compression, or for the production of a composite gasoline fraction for blending with other gasoline fractions of lower critical compression for the production therefrom of motor fuel gasolines having a high critical compression.

The receiver 1, the scrubbing tower 4, and the rectifying tower 5 may be operated, for example, as described in an application filed December 16, 1929. Serial Number 414,419, by Eugene C. Herthel.

Other absorbent media, instead of the gasoline condensate separated in the receiver 1, however, may be used for the purpose of recovering the unsaturated hydrocarbon constituents from the gas mixture separated in the receiver 1. For example, this gas mixture may be subjected to a conventional scrubbing treatment with an absorbent oil and the absorbed unsaturated hydrocarbon constituents distilled therefrom subjected to rectification for the production of a condensate con-

taining unsaturated hydrocarbon constituents in high concentration to be supplied to the mixing pump 10 through connection 19.

The gas mixture discharged through connection 15 may be subjected to scrubbing treatment, for the further recovery of unsaturated hydrocarbon constituents, with sulfuric acid to be supplied to the mixing pump 10 through connection 24 as described in an application filed December 16, 1929, Serial Number 414,362, by Frank A. Apgar.

The following example will further illustrate the process of the invention: gas oil is heated to a cracking temperature approximating 1080° F. under a pressure approximating 100 pounds per square inch and the resulting hot oil products are subjected to fractionation to separate a gasoline fraction and associated low boiling vapors and gases. This gasoline fraction is subjected to condensation and the resulting gasoline condensate and gas mixture are separated. The separated gas mixture is subjected to a scrubbing treatment at a temperature approximating 80° F. under a pressure approximating 250 pounds per square inch with the separated gasoline condensate. The resulting gasoline condensate mixture is subjected to rectification under a pressure approximating 110 pounds per square inch producing a vapor mixture containing unsaturated hydrocarbon constituents in high concentration and producing a rectified gasoline condensate having a relatively low vapor pressure. The vapor mixture is condensed and the condensate

treated with 60 per cent. by volume of 80 per cent.  $H_2SO_4$  sulfuric acid at a temperature approximating 80° F. and at a pressure approximating 150 pounds per square inch. The products of the resulting reaction are separated into a composite oil mixture and a composite acid mixture.

The composite oil mixture is neutralized with caustic soda and a composite polymerized gasoline fraction is distilled therefrom. The composite acid mixture is diluted with 200 per cent. by volume of water and a composite polymerized oil fraction is distilled therefrom and a composite polymerized gasoline fraction is redistilled from this distillate in the presence of caustic soda. In this manner 40-50 per cent. of a rectified gasoline condensate, 1-2 per cent. of a composite polymerized gasoline fraction and 2-4 per cent. of a composite oxidized gasoline fraction may be recovered from the original gas oil.

In carrying out the process of the invention, no separation of the several unsaturated hydrocarbon constituents of the liquefied hydrocarbons subjected to the treatment with sulfuric acid is necessary and any necessity for critical control of the acid treatment to avoid polymerization reactions and to maintain conditions appropriate to sulfating re-

actions is also avoided. Thus, although the process of the invention embodies some elements of operation analogous to operations carried out for the production, for example, of alcohols from hydrocarbon gas mixtures, it is essentially different from such operations in eliminating features of operation which tend to increase operating expense to a point prohibitive in the manufacture of motor fuel gasoline.

I claim:

1. In the manufacture of motor fuel gasoline having a high critical compression, the improvement which comprises subjecting a high boiling hydrocarbon oil to a cracking temperature upwards of 950° F. and separating a gas mixture including unsaturated hydrocarbon constituents from the products of the cracking operation, subjecting a hydrocarbon composite including the unsaturated hydrocarbon constituents of this gas mixture to treatment with sulfuric acid, separating the resulting composite acid mixture and composite oil mixture, distilling a polymerized gasoline fraction from the separated composite oil mixture, hydrolyzing the separated composite acid mixture to produce a second composite oil mixture, distilling an oxidized gasoline fraction from this second composite oil mixture, and combining the composite polymerized gasoline fraction and the composite oxidized gasoline fraction so produced with a gasoline fraction of lower critical compression to produce a motor fuel gasoline having a high critical compression.

2. In the manufacture of motor fuel gasoline having a high critical compression, the improvement which comprises subjecting a high boiling hydrocarbon oil to a cracking temperature upwards of 950° F. and separating a gasoline condensate and a gas mixture including unsaturated hydrocarbon constituents from the products of the cracking operation, subjecting a hydrocarbon composite including the unsaturated hydrocarbon constituents of this gas mixture to treatment with sulfuric acid, separating the resulting composite acid mixture and composite oil mixture, distilling a polymerized gasoline fraction from the separated composite oil mixture, hydrolyzing the separated composite acid mixture to produce a second composite oil mixture, distilling an oxidized gasoline fraction from this second composite oil mixture, and combining the composite polymerized gasoline fraction and the composite oxidized gasoline fraction so produced with the gasoline condensate to produce a motor fuel gasoline having a high critical compression.

In testimony whereof I affix my signature.  
HARRY L. PELZER.